

## UNITED STATES PATENT OFFICE

2,116,583

## WETTING AGENTS USEFUL FOR ALKALINE MERCERIZING SOLUTION

Ferdinand Münz, Frankfort-on-the-Main, Germany, assignor to General Aniline Works, Inc., New York, N. Y., a corporation of Delaware

No Drawing. Application March 31, 1936, Serial No. 71,875. In Germany April 11, 1935

## 4 Claims. (Cl. 8—20)

My invention relates to wetting agents useful for alkaline mercerizing solutions, more particularly those corresponding to the general formula:



wherein  $\text{R}_1$  and  $\text{R}_2$  stand for alkyl groups, the total number of carbon atoms in both said groups being at least 3 and no more than 8 carbon atoms and Me means an alkali metal.

Insofar as they are sufficiently soluble in alkaline mercerizing solutions, they may be used as wetting agents either alone or in admixture with substances which are less soluble per se, but the solubility and effect of which is increased by the simultaneous presence of the above sulfaminic acids. Insofar as the sulfaminic acids of the above formula are not sufficiently soluble in strong alkaline solutions, they may be dissolved therein by the addition of the well known dispersing agents.

The present sulfaminic acids are obtainable by acting with the usual agents, such as sulfur trioxide, chlorosulfonic acid, amidosulfonic acid and the like, on secondary amines of the formula:



$\text{R}_1$  and  $\text{R}_2$  having the above signification.

Compared with sulfaminic acids of primary amines and fatty acid amides, described in the literature (cf. German Patent No. 572,283), which are characterized by the presence of alkyl groups containing more than 8 carbon atoms in their molecule, the present sulfaminic acids are superior as to their wetting effect for alkaline mercerizing solutions. Compared with the corresponding amides of the dithiocarbonic acid (cf. U. S. Patent No. 2,043,329), the present sulfaminic acids have the advantage of being insensible towards metallic salts and the contact with metals, particularly copper.

In order to illustrate my invention the following examples are given, the parts being by weight and all temperatures in Centigrade degrees. I wish it however to be understood that my invention is not limited to the particular products nor reaction conditions mentioned therein.

## Example 1

To a mercerizing solution of 30° Bé. 0.3% of

the sodium salt of the di-n-propyl-sulfaminic acid of the formula:



are added. Raw cotton is nearly immediately wetted.

By adding organic solvents, bases, naphthenic or aliphatic acids and other substances insoluble per se in mercerizing solutions the wetting and shrinking effect can be increased.

## Example 2

15 parts of the sodium salt of the di-isobutyl-15 sulfaminic acid of the formula:



are dissolved in 100 parts of technical xyleneol 25 and about 7 parts of crude xylene are added. When adding only 5 grs. of this mixture to a liter of a mercerizing solution a very rapid shrinking of raw cotton is obtained.

Instead of the sodium salt of the above sulfaminic acid one may use the sodium salt of the monoethyl-monoisobutyl-sulfaminic acid of the formula:



## I claim:

1. A composition of matter comprising an alkaline mercerizing bath containing a compound of the general formula:



wherein  $\text{R}_1$  and  $\text{R}_2$  represent alkyl groups the total number of carbon atoms in the two alkyl groups ranging from 3 to 8 and Me means an alkali metal.

2. A composition of matter comprising an alkaline mercerizing bath containing a compound of the general formula:  $\text{MeO}_3\text{S}-\text{N}-(\text{R}_1)_2$ , 55

wherein  $R_1$  stands for an alkyl group containing from 2 to 4 carbon atoms and Me means an alkali metal.

3. A composition of matter comprising an alkaline mercerizing bath containing a compound of the general formula:



wherein Me means an alkali metal.

4. A composition of matter comprising an al-

kaline mercerizing bath containing a compound of the general formula:



10

wherein Me means an alkali metal.

FERDINAND MÜNZ.